

## UNITED STATES PATENT OFFICE

DAVID R. MERRILL, OF LONG BEACH, CALIFORNIA, ASSIGNOR TO UNION OIL COMPANY OF CALIFORNIA, OF LOS ANGELES, CALIFORNIA, A CORPORATION OF CALIFORNIA

## SOLUBLE OIL CONTAINING ETHER DERIVATIVES OF POLYHYDROXY ALCOHOLS

No Drawing. Application filed January 4, 1928. Serial No. 244,562.

This invention relates to the production of the so-called "soluble" oils which disperse readily when added to water for the preparation of sprays, dips, cutting oils and the like.

In producing these soluble oils, a neutral oil, which commonly is of mineral origin, and a soap are employed in conjunction with a common solvent or blending agent. Sodium naphthenate or other soap of the same type may be employed as the soap required, and while the present invention is not limited to the use of a naphthenate it is especially adapted thereto.

The chief object of the invention is to employ a common solvent or blending agent which shall possess better blending power for the soap and oil than has been known heretofore, and one which shall at the same time have a more pleasant and less pronounced odor than often obtained in the past. This agent, in a preferred form, should be particularly suitable for employment with an alkali metal naphthenate such as sodium naphthenate, and since such an agent is also suitable where other alkali metal soaps are used it may therefore be employed with either the naphthenates or said other soaps.

In working upon soluble oils, I have found that the common solvent for the soap and oil should be of such character as to bring the soap into a practically true solution in oil in the cold, as distinguished from a colloidal solution or jelly. For soaps of the sodium naphthenate type, the common solvent employed should be partly soluble in water but not miscible therewith in all proportions, due to the fact that a solvent which is miscible with water in all proportions will largely leave the oil and dissolve in water when the soluble oil is poured into water, thus leaving the soap and oil in a form which will not readily disperse in the water. In other words the blending agent employed must be soluble in the oil and must also have solubility in water, and a more or less careful balance must be maintained in these solvent properties. This balance I have found to be advantageously effected by the inclusion of an ether group in the molecule of a poly-

hydroxy-alcohol, whereby there is present in the solvent a hydroxyl group to lend solubility in water and an ether group to promote solubility in oil at the same time. A compound of this character has high solvent power for the soaps. Such hydroxy-ethers may be of several types, for instance, mono-ether derivatives of the glycols or diether derivatives of glycerol; or, otherwise stated, any ether derivative of a polyhydroxy-alcohol which derivative contains at least one free hydroxyl and which possesses the required solubility. This applies particularly to the lower polyalcohols, and opens up the field to those hydroxy-ethers of the lower alcohols which are soluble to some extent in both oil and water.

Thus, the invention in a broad aspect resides in the preparation of a soluble oil from a neutral oil (animal, vegetable or mineral) and sodium naphthenate or other soap, by means of a blending agent in the form of a hydroxy-ether which is a common solvent for both the oil and soap and possesses limited solubility in water. More particularly the common solvent is one which will act to bring the soap into a substantially true solution in the oil. In a preferred form this common solvent or blending agent is an ether derivative of a polyhydroxy-alcohol which derivative contains a free hydroxyl and possesses the solvent properties stated. For the most part this places the alcohol base in the class of the polyhydroxy-alcohols having a maximum of four hydroxyl groups, it being important only that the proper solubility be maintained.

Considering the invention in greater detail, the soluble oil is produced by treating soap and a neutral oil with a common solvent which acts as a blending agent. The soap may be sodium naphthenate or other alkali metal naphthenate or other alkali metal soap, these soaps as is well known, all being soluble in water; the oil may be of animal, vegetable or mineral origin; and the solvent will be one which has a mild pleasant odor, which is partially miscible with water, and which is capable of bringing the soap into a true or nearly true solution in the oil while

55

60

65

70

75

80

85

90

95

100

cold, as shown by the very low viscosity of the product, and as distinguished from a colloidal solution or a colloidal jelly. This solvent or blending agent thus is a common solvent for water, the oil and the soap. A small quantity of such a blending agent will produce a solution of a relatively large quantity of soap in the oil, as much as one part of soap being brought into solution in about 10 three parts of oil by about one-fifth part of blending agent. As indicated above the best results are obtained, especially with soaps of the sodium naphthenate type, when the common solvent is somewhat soluble in water but not miscible in all proportions. The reason for this is to prevent the solvent from leaving the soluble oil and dissolving in water when the oil is poured into water and thus leaving the soap and oil behind so that 15 ready dispersion is impossible, as will happen when one employs a solvent which is miscible in all proportions in water, such as ethyl-alcohol.

Thus, to insure proper solubility in the 20 oil and also in water, especially where the naphthenates are employed, a careful balance must be established. This can be accomplished by using an agent which contains an hydroxyl group and an ether group, 25 the hydroxyl group lending water solubility and the ether group lending oil solubility, such a compound not being wholly soluble in water and at the same time offering high 30 solubility for the soap employed. Such substances are hydroxy-ethers, and all those 35 hydroxy-ethers which possess the requisite solvent properties above outlined are suitable agents. This class is defined as those derived from polyhydroxy-alcohols having 40 not more than four hydroxyl groups. Alcohols having a greater number of hydroxyls have molecular weights that are too high to 45 yield the desired solvent properties. Thus, hydroxy-ethers which have such desired properties are ether derivatives of the lower polyhydroxy-alcohols particularly the dihydroxy-alcohols (glycols) and the trihydroxy-alcohols such as glycerol. Specific examples in 50 these groups are monoethyl-ether of ethylene glycol and dipropyl-ether of glycerol. Other monoethers of ethylene glycol may be used as well as monoethers of other glycols. Likewise, similar derivatives of glycerol besides dipropyl-ether may be used as well as others 55 of the trihydroxy-alcohols, as long as a free hydroxyl group remains. Some other radical than the ether group may be introduced in 60 place of one of the ether groups in glycerol, thus retaining an ether group for oil solubility and a hydroxyl group for water solubility. A diether formed by substituting two 65 ether groups for two of the four hydroxyls of erythritol may be used, and so on so long as the series does not become so high that 70 the desired solubility is lost, or the ether

groups are not so overbalanced in number by hydroxyl groups that the water solubility becomes excessive as compared with the oil solubility and effectively destroys the desired function of the ether groups. Monoethers of the glycols present a particularly satisfactory group which includes the mono-methyl, 75 ethyl, propyl and butyl ethers of ethylene glycol or of propylene glycol.

All of these solvents possess the desired properties above mentioned of blending or bringing into solution a relatively large quantity of soap with the oil by employing only a relatively small quantity of the blending solvent, and the solution so produced is a 80 true solution of the soap in the oil as established by the low viscosity of the mixture. The resulting soluble oil emulsifies freely and disperses readily upon dilution with water in all proportions.

As a specific example, a sodium naphthenate was used which had been prepared by neutralizing naphthenic acid with sodium hydroxide solution (for example 40° Bé.) and heating the soap thus formed to drive off most of the water, the water content being reduced to somewhat less than 8%. To 25 parts of this soap there was added 70 parts of neutral mineral oil and 5 parts of monoethyl-ether of ethylene glycol, the ether being introduced at a temperature of about 120° F. to avoid excessive evaporation. The product was a homogeneous oily material of low viscosity which emulsified readily in water with little or no agitation and in all 100 proportions.

Results such as this are always obtained unless too much water has been left in the soap, 8% or less of water being a sufficiently small amount. The presence of excessive water is 105 indicated by lack of homogeneity of the soluble oil mixture.

Various oils may be used in preparation of the product desired, for example, light oils such as kerosene, or heavy oils such as crude oil or heavy lubricating oil, the resulting products emulsifying readily in water and the emulsions remaining stable under all degrees of dilutions. Corresponding results may be obtained with vegetable oils such as 110 cotton seed oil, or animal oils such as fish oils, or mixtures of these with each other or with mineral oil, although emulsions formed from oils of purely mineral origin are in general 115 the most stable.

Soluble oils prepared according to the foregoing pass all government tests including the corrosion and odor tests, and since the common solvents described are unusually effective as blending agents for the soap and oil the required amount of such solvents is somewhat smaller. Thus the blending features and the improved odor present very desirable advantages.

It is to be understood that the above disclosure

sures are not to be considered as limiting but merely as illustrative of the generic invention, and that many variations may be made within the scope of the claims.

5 I claim:

1. A soluble oil comprising an oil containing in solution a soap and a hydroxy-ether soluble in both the oil and water.

10 2. A soluble oil according to claim 1 wherein the soap is a naphthenate.

15 3. A soluble oil comprising an oil, a soap and a blending agent in the form of an ether derivative of a polyhydroxy-alcohol which derivative retains a free hydroxyl and which derivative is soluble in both the oil and water.

20 4. An oil according to claim 3 wherein the soap is a naphthenate.

25 5. A soluble oil according to claim 3 wherein the oil employed is a mineral oil.

30 6. A soluble oil comprising a neutral oil, a naphthenate soap and a common solvent in the form of a hydroxy-ether which is at least partly soluble in the oil but only partly miscible with water.

35 7. A soluble oil comprising an oil, a soap and a common solvent capable of bringing the soap into a practically true solution in the oil, said solvent being a hydroxy-ether of a polyhydroxy-alcohol and having solubility being partly soluble in water.

40 8. A soluble oil comprising an oil, a soap and a blending agent in the form of a hydroxy-ether derived from a polyhydroxy-alcohol which originally contained from two to four hydroxyls.

45 9. A soluble oil comprising a mineral oil, a naphthenate ~~and~~ and monoethyl-ether of ethylene glycol.

50 10. A soluble oil comprising an oil, a soap and a blending agent in form of a monoether of a glycol.

55 11. A soluble oil comprising a solution of approximately 5 parts of neutral oil, 1 part of a soap and  $\frac{1}{6}$  part of a blending agent containing an ether group to impart solubility in the oil and a free hydroxyl to impart solubility in water.

60 12. A soluble oil comprising approximately 5 parts of mineral oil, 1 part of naphthenate soap and  $\frac{1}{6}$  part of a blending agent which is an ether derivative of a polyhydroxy-alcohol, the derivative containing a free hydroxyl group and having both oil and water solubility.

65 13. A soluble oil according to claim 1 wherein the soap is soluble in water.

70 14. A soluble oil according to claim 1 wherein the soap is an alkali metal naphthenate.

75 15. A soluble oil comprising a neutral oil, a water soluble soap, and a monoether of a glycol serving as a blending agent and soluble in both oil and water.

80 16. Soluble oil according to claim 15 wherein the soap is an alkali metal naphthenate.

Signed at Wilmington, in the county of Los Angeles and State of California, this 19th day of December, A. D. 1927.

DAVID R. MERRILL.

70

75

80

85

90

95

100

105

110

115

120

125

130